

## UNITED STATES PATENT OFFICE

2,173,430

PIGMENTED BASE FOR PAINTS AND THE  
LIKE

Max Raymond Vogel, Easton, Pa., assignor to  
Binney and Smith Company, New York, N. Y.,  
a corporation of New Jersey

No Drawing. Application July 16, 1937,  
Serial No. 154,103

10 Claims. (CL 260—40)

This invention relates to improvements in pigmented bases for use in the manufacture of paints, varnishes, lacquers, enamels, inks, plastics and the like, and more particularly aims to provide an improved process for the permanent colloidal dispersion of pigments within a resinous or similar vehicle, together with the products thereof.

It is essential in the preparation of a satisfactory paint or pigmented plastic to properly disperse the pigment particles throughout the vehicle. Various methods and machines have been devised for the mechanical manipulation of mixtures of the pigment and vehicle to produce a thorough and uniform dispersion but no single method has proven completely successful. The more common machines used are the ball and pebble mills, dough mixers, two roller mills, three roller mills and stone mills. Many addition agents have been suggested which when used in combination with the various mechanical means of grinding somewhat improve the resulting product. These agents appear to be specific to the type of vehicle chosen; that is, an agent which may operate satisfactorily with nitrocellulose may not function with a synthetic resin, and vice versa.

It has now been discovered that if the pigmentation of a solid, water-insoluble resin is conducted in the presence of a stable organic amine containing a plurality of —NH<sub>2</sub> groups, unusually good, stable dispersions are obtained. Coating compositions prepared from these dispersions or pigmented bases exhibit, when applied to the surface to be coated, a much higher gloss and a more pronounced depth of color than is the case when such polyamines are omitted.

The process of pigmentation is preferably conducted by a two-step process corresponding to that disclosed in the patent of William B. Wiegand, No. 2,045,006, dated June 23, 1936. In the first step of this process the dispersion medium, preferably an alkyd resin vehicle, is coalesced, agglomerated, agglutinated or massed with a pigment, for example carbon black, and with the polyamine under conditions most favorable to ready mixing, and either with or without the application of high shearing stresses, such as are produced by passing the mass between pressure rolls of the type commonly used in the rubber industry. In the second step of the process the mass resulting from the initial treatment is subjected to unusually high shearing stresses, these high shearing stresses being obtained by subject-

consistency to very strenuous mechanical manipulation.

The stable organic amine may be incorporated at any point prior to or during the colloidal dispersing of the pigment in the medium. Stable organic amines containing a plurality of unsubstituted —NH<sub>2</sub> groups found most suitable for this purpose are triethylenetetramine, meta-phenylenediamine, diethylenetriamine, ethylenediamine, metatoluylendiamine and benzidine. By the term "amine" it is not intended to include amido type compounds of the nature of urea and its derivatives, such as guanidine. This latter compound, guanidine, furthermore is unsuitable for use in pigmented bases because of its relative instability. Nor is it intended to include within the scope of the invention the use of such insoluble or complex organic compounds as, dyes which contain a plurality of amino groups of the substituted type. The quantity of polyamine can be varied over a broad range but it has been found that proportions between one and fifteen percent have the most beneficial effect in dispersing the pigment. While the free amines produce the most desirable results, the soaps of such amines may be used with some success.

The Wiegand two-step process of pigmentation referred to above is to be distinguished from the other commonly employed methods of dispersing pigment in paint media, in that the massed pigment and vehicle mixture in the Wiegand process is in a stiffly plastic or "leather-like" condition and is subjected to exceptionally high shearing stresses. Neither of these conditions exist in the other processes, since the mixture of pigment and vehicle is usually in a condition ranging from relative liquidity in ball or stone mill grinding to a "rubbery" or flexibly plastic condition in the dough mixer or the two roller (rubber) mill grinding. This relatively fluid or soft plastic condition, resulting from the addition of solvents, plasticizers, softeners, soft resin and the like to the vehicle and pigment mixture, prevents the application of high shearing stresses which are essential in preparing relatively complete and permanent colloidal dispersions of the pigment in the vehicle.

The "leather-like" consistency of the plastic

mass in the Wiegand process corresponds in general to the stiffness of sole leather.

My invention will be more clearly understood from the following examples of the mode of preparing a concentrated pigmented base following generally the mechanical procedure described in the above-mentioned Wiegand patent.

*Example I*

10 A typical charging composition for a black pigmented alkyd resin base is as follows:

| Parts by weight                                                    |     |  |
|--------------------------------------------------------------------|-----|--|
| Alkyd resin modified with 50% drying oil fatty acids (acid No. 53) | 500 |  |
| 15 Carbon black                                                    | 300 |  |
| Textile spirits                                                    | 215 |  |
| Triethylenetetramine                                               | 30  |  |

20 In the first step of preparing the base the above ingredients may be massed by passing between the pressure rolls of a roller mill of the general type used in the rubber industry. The mixture is repeatedly passed between the rolls while the resin vehicle is in a viscous plastic condition until the pigment and polyamine have been suitably distributed throughout the resin, and the combined product has reached the degree of consistency best adapted for the application thereto of high shearing stresses. Alternatively, or prior thereto, the mixture of ingredients may be massed in a mixer such as a dough mixing machine.

25 The petroleum hydrocarbon solvent, textile spirits, in the above formula is used simply to wet down the carbon black pigment, and evaporates substantially completely during the process.

30 In the second step the resin vehicle, having the carbon black and polyamine incompletely dispersed therein and being of a stiff plastic or leather-like consistency, is passed between the same or a second pair of pressure rolls set closely together, the function of which rolls is to subject the mass to exceptionally high shearing stresses. The leather-like consistency of the mass being operated upon may be maintained, if necessary, by heating or cooling the rolls. The rolls are suitably driven at different speeds so as to increase the shearing stresses and are set tight so that when the mass is passed through the rolls it is sheeted out to a thickness of about one-sixteenth to one thirty-second inch. The sheets issuing from the rolls may be repeatedly passed between the rolls until a thorough and permanent colloidal dispersion of the pigment in the resin medium is assured.

35 These pigmented sheets, from the Wiegand process, at normal room temperature will usually be brittle permitting the same to be broken into flaky fragments of paper-like thinness, which when dissolved in a suitable solvent with or without additional ingredients will form a paint, varnish, enamel or lacquer possessing an unusual depth of coloring, a high lustre and an exceptional degree of permanency.

40 The drying oil fatty acid modified glycerol phthalate resin in the above example is sold under the trade name of "Rezyl #110". Other drying oil fatty acid modified alkyd resins may be substituted for this resin such as a 29% modification which has an acid number of about 57 and which is available under the trade name "Rezyl #1102". These resins are made in accordance with the procedure outlined in the U. S. Patents 1,893,873 and 1,893,874 to Kienle and Adams respectively. Pure alkyd plastic resins

45 free from phenol and resin modifying agents such as "Beckosol #7" may also be used. This latter resin has a low acid number ranging from about five to ten. Alkyd resins modified with saturated fatty acids such as "Rezyl #12" which is modified with 28% non-drying fatty acids and has an acid number of 24, likewise may be substituted for or used in combination with the alkyd resin in Example I. Pigmented bases prepared with "Rezyl #12" are generally compatible with nitro-cellulose compositions. Natural resin or rosin or other modified alkyd resins such as the "Teglacs" and "Beckosol #1" may also be used in preparing these pigmented bases.

50 Other water-insoluble resins than the alkyd resins such as the phenol-aldehyde, urea-aldehyde and the coumarone-indene resins and even the natural and modified natural resins may replace or be combined with the foregoing alkyd resins. "Beckacite #1001" is a phenolic resin 20 which has been found satisfactory in preparing the improved pigmented bases. Rosin, ester gum and "Amberol 801" will also function satisfactorily in the process.

55 Although the invention is especially applicable 25 to the manufacture of carbon black pigmented bases, other common color pigments, for example, Prussian blue, organic maroons and titanium dioxide, may be substituted for or be used with carbon black in combination with the resin and 30 polyamine. The following examples show charging combinations for other pigments than carbon black.

*Example II*

60 A grinding composition for a grey pigmented resin base is as follows:

| Parts by weight                                                  |      |    |
|------------------------------------------------------------------|------|----|
| Alkyd resin modified with 28% non-drying fatty acids (Rezyl #12) | 500  | 40 |
| Antimony oxide                                                   | 3700 |    |
| Carbon black                                                     | 80   |    |
| Textile spirits                                                  | 215  |    |
| Triethylenetetramine                                             | 30   |    |

*Example III*

65 A typical blue charging composition is as follows:

| Parts by weight                                                     |     |    |
|---------------------------------------------------------------------|-----|----|
| Alkyd resin modified with 29% unsaturated fatty acids (acid No. 57) | 500 | 50 |
| Prussian blue (C. P. non-bronzing type)                             | 600 |    |
| Textile spirits                                                     | 215 |    |
| Triethylenetetramine                                                | 30  |    |

70 Both of these compositions are treated according to the procedure of Example I. The alkyd resin can of course be replaced by other type resins as indicated above. Other polyamines may be used in place of or in combination with the triethylenetetramine.

75 The flaky fragments of the pigmented resin base if made from a non-oxidizing resin may be marketed in bulk or in packages or cans. However, when the resin employed in the preparation 80 of the base is susceptible to oxidization, such as the drying oil modified alkyd resins, the pigmented base is combined with a suitable solvent such as toluene in a dough mixer to form a paste or solution. The paste is usually prepared so that it contains between 50 and 60 percent solids. Either the dry flake or the paste may be added to any liquid vehicle with which the resin in the base is compatible, in preparing a coating composition.

The pigmented bases corresponding to those disclosed in Examples I, II and III above may be dissolved in a liquid vehicle so as to form resin or cellulose derivative coating compositions having the following formulae. In the following examples the fatty acid modified alkyd resin pigmented base is composed of 50 percent solids and 50 percent of toluene.

## RESINOUS ENAMELS

10

## Example IV

Parts by  
weight

|                                                              |      |
|--------------------------------------------------------------|------|
| Fatty-acid modified alkyd resin pigmented<br>base            | 130  |
| Toluene                                                      | 210  |
| Phenol and oil modified alkyd resin solution<br>(50% solids) | 840  |
| Drier solution                                               | 20.7 |

20 The phenol modified alkyd resin solution mentioned above may be the grade sold under the trade name of "Beckosol #1 Solution" which is cut with equal parts of mineral spirits. The acid number is between 10 and 15.

25

## Example V

Parts by  
weight

|                                                                                    |      |
|------------------------------------------------------------------------------------|------|
| Fatty-acid modified alkyd resin pigmented<br>base                                  | 130  |
| Toluene                                                                            | 350  |
| Alkyd resin modified with 37% drying oil<br>fatty acids and 14% rosin (60% solids) | 700  |
| Drier solution                                                                     | 20.7 |

30 The alkyd resin recited above is marketed under the trade name of "Rezyl Solution J (114)". The acid number of this resin is 33.

35 The toluene referred to in these two examples may be replaced by any of the common organic liquids used in such resinous enamels, namely coal tar solvents such as xylene, solvent naphtha and benzene; petroleum solvents such as white spirits, "Solvesso" and petroleum spirits; turpentine and the alcohols such as butyl alcohol.

40 The proportion of drier solution can be varied over wide limits depending on the type finish desired, that is, whether low bake, high bake or air-dry. The drier used in the above example 50 contains about .145 gram of metal for each gram of solution. The composition of the drier is as follows:

## Example VI

Parts by  
weight

|                                                     |    |
|-----------------------------------------------------|----|
| Cobalt naphthenate in mineral spirits (6%<br>metal) | 22 |
| Lead naphthenate in mineral spirits (34%<br>metal)  | 39 |
| Xylene                                              | 39 |

100

## NITROCELLULOSE LACQUER

65

## Example VII

Parts by  
weight

|                                                                |     |
|----------------------------------------------------------------|-----|
| Fatty-acid modified alkyd resin pigmented<br>base (Example II) | 100 |
| Butyl alcohol                                                  | 200 |
| Nitrocellulose solution (25% solids)                           | 800 |
| Alkyd resin modified with 28% non-drying<br>fatty acids        | 100 |
| Dibutyl phthalate                                              | 68  |

In the above example it will be understood that all solvents, plasticizers, resins, etc., are compatible with nitrocellulose solutions. The alkyd resin mentioned above is sold in the trade under the name of "Rezyl #12".

5 While in the specific examples given above alkyd resins are employed, it will be understood that in a broader sense the pigmented base is not limited to use with alkyd resins but other compatible paint and lacquer ingredients such as resins, natural or synthetic, cellulose derivatives and oils may be substituted for or used in combination with the alkyd resins. Other synthetic resins which may be used in the coating compositions include "Beckolin", "Amberol 801", "Glyptal Solution #2452" and "Beckosol #1323".

15 The stable organic polyamine is preferably added to the mixture of resin and pigment while agglomerating these materials but may be incorporated therein at any point in the process so 20 long as it is present as a free amine when the pigment is to be colloidally dispersed in the plastic mass.

25 Although the invention is best practiced by employing the two-step mechanical treatment disclosed in the above-mentioned Wiegand patent by which the most striking and unusual results are attained, it is nevertheless within the contemplation of my invention in its broad aspects to employ the stable organic primary polyamine 30 with other modes of pigment dispersion in a resin while the later is in a solid plastic state. Softer resins can of course be used with these other methods of pigmentation since the stiffly plastic condition is not employed in such processes and 35 the flaked pigmented base is not produced.

30 The present invention is not to be restricted to any specific proportions or manner of procedure beyond the limitation of the appended claims.

40 I claim:

1. A pigmented resin base comprising a ground intermixture of a pigment with a solid, plastic, water-insoluble resin and a stable, soluble, organic amine containing a plurality of unsubstituted —NH<sub>2</sub> groups, said amine serving as 45 a dispersing agent for the pigment.

2. A pigmented resin base comprising a ground intermixture of carbon black with a solid, plastic, water-insoluble resin in the presence of a stable, soluble, organic amine containing a plurality of 50 unsubstituted —NH<sub>2</sub> groups, said amine serving as a dispersing agent for the carbon black.

3. A pigmented resin base comprising a pigment uniformly massed and mechanically worked with a solid, plastic, water-insoluble resin and a 55 stable, soluble, organic amine containing a plurality of unsubstituted —NH<sub>2</sub> groups, said amine serving as a dispersing agent for the pigment.

4. A pigmented resin base comprising carbon black uniformly massed and mechanically worked 60 with a solid, plastic, water-insoluble, alkyd resin and a stable, soluble, organic amine containing a plurality of unsubstituted —NH<sub>2</sub> groups, said amine serving as a dispersing agent for the carbon black.

5. A pigmented resin base comprising carbon black uniformly massed and mechanically worked with a solid, plastic, water-insoluble, fatty-acid modified alkyd resin and ten percent triethylenetetramine based on the weight of the carbon 70 black, said triethylenetetramine serving as a dispersing agent for the carbon black.

6. A pigmented resin base comprising a color pigment uniformly massed and mechanically worked with a solid, plastic, water-insoluble, 75

rosin-modified alkyd resin and metaphenylenediamine, said metaphenylenediamine serving as a dispersing agent for the pigment.

7. A pigmented resin base comprising carbon black uniformly massed and mechanically worked with a solid, plastic, water-insoluble, synthetic resin and diethylenetriamine said diethylenetriamine serving as a dispersing agent for the carbon black.

10. A high gloss resin enamel including a solution of a pigmented resin base, said pigmented resin base comprising a ground intermixture of a pigment with a solid, plastic, water-insoluble resin and a stable, soluble, organic amine containing a plurality of unsubstituted  $-\text{NH}_2$  groups, said amine serving as a dispersing agent for the pigment.

9. A high gloss resin enamel including a solu-

tion of a pigmented resin base, said pigmented resin base comprising carbon black uniformly massed and mechanically worked with a solid, plastic, water-insoluble, alkyd resin and a stable, soluble, organic amine containing a plurality of 5 unsubstituted  $-\text{NH}_2$  groups.

10. A grey nitro-cellulose lacquer including an organic solvent solution of nitrocellulose, synthetic resin, plasticizer and a grey pigmented base, said pigmented base comprising carbon 10 black, antimony oxide, and triethylenetetramine uniformly massed and mechanically worked with a solid, plastic, water-insoluble, fatty-acid modified alkyd resin which is compatible with nitrocellulose, said triethylenetetramine serving as a 15 dispersing agent for the carbon black.

MAX RAYMOND VOGEL.